

## UNITED STATES PATENT OFFICE

2,246,166

SINTERED HARD-METAL ALLOY FOR  
IMPLEMENTS AND TOOLS

Walther Dawihl, Berlin-Kohlhasenbruck, and  
Karl Schröter, Berlin, Germany, assignors to  
General Electric Company, a corporation of  
New York

No Drawing. Application March 30, 1940, Serial  
No. 326,972. In Germany February 2, 1939

2 Claims. (Cl. 75—136)

Hard metal alloys or cemented carbides heretofore produced generally have consisted of one or more hard metal carbides with a high melting point such as tungsten carbide, molybdenum carbide, titanium carbide or tantalum carbide and a metallic addition, the so-called auxiliary metal which has a relatively low melting point and may constitute up to about 25% of the weight of the hard metal alloy. Cobalt, nickel or iron either individually or in suitable mixture preferably are used for such metallic additions and these metals are very soft as compared to the hard metal carbides. As a result of this great difference in hardness it sometimes happens that in the use of hard metal alloy tools of the above-noted character, the auxiliary metal wears away relatively quickly thereby exposing the hard carbide grains which thereafter break away from the tool and shorten its life.

According to the present invention, this property of hard-metal composition which reduces the life of the tool or implement, is improved when a mixture, preferably pre-heated and crushed again, consisting of a metal with a lower melting point or several such metals, as cobalt, nickel, iron, manganese or chromium and a tungsten or molybdenum carbon alloy with a carbon content between 1 and 5% is used as the addition to the carbide or carbides of metals with a high melting point which forms the basic mass. The portion of the admixture of more readily melting metals lies in that case between 10 and 80%; consequently the portion of the tungsten or molybdenum carbon alloy is from 90 to 20%. Such mixtures have melting points which lie between 1400° and 1600° irrespective of which of the more readily melting auxiliary metal is used and irrespective of whether the carbon content of the tungsten or molybdenum carbon alloy present in the mixture is only 1% or up to 5%. Because of the relatively low melting temperature of the added mixture, it is possible to retain the sintering temperatures customary in the hard-metal industry when using the new admixture, and to obtain thereby all advantages which are included in the application of auxiliary metals with a lower melting point. On the other hand, it has, however, been found that the admixtures that are to be used according to the invention within the indicated range of composition have much higher hardness values than the pure auxiliary metals generally used heretofore. The hardness values of the indicated mixtures of addition are sometimes so high that, if desired, they may be utilized independently as hard alloys.

Their inherent hardness closely approaches the inherent hardness of the carbides that form the basic compound of the entire composition so that the wearing away phenomena hereinbefore described is avoided.

To obtain the highest hardness values, it is particularly advantageous to employ composition of the added mixture which lie within the range of composition indicated by the formulas

10  $\text{Co}_6\text{W}_2\text{C}$  and  $\text{Co}_3\text{W}_3\text{C}$ .

In the production of the added mixture, it is desirable to mix about 35 parts by weight of cobalt with about 65 parts by weight of a tungsten carbon alloy having a 3% carbon content. 15 The mixture is heated to approximately 1300° C. to give the alloy an opportunity to form and is then pulverized. Of this pulverized alloy there are then mixed 10 parts by weight with 90 parts by weight of tungsten carbide having a carbon content of 6.12%. Molded bodies are produced from the mixture and these are then sintered in a known manner at a temperature of approximately 1500° C.

The sintered bodies obtained are distinguished 25 by a hardness which is distributed very uniformly over the entire cross section; their strength is somewhat less than that of hard metal alloys produced with pure alloy metals so that they may be used to advantage whenever a uniformly high 30 hardness is required without too high strength requirements. The alloy formation between the carbide or carbides that constitute the basic mass and the added mixture is favored considerably when the latter, prior to the mixing with the 35 basic mass, is preheated and crushed again. The more ready alloy formation in conjunction with the uniform distribution of the particles of the added mixture in the basic carbide mass results in finished sintered bodies which have an extremely low degree of porosity.

It previously has been suggested to add to the 45 initial materials of hard metal alloys, metals with a high melting point like, for instance, metallic tungsten. However, it has been found that the conversions which occur during the sintering, lead to alloys whose distribution in the sintered body is very irregular so that in the structure of the finished sintered body, a pronounced concentration in this alloy can be found at individual points, while it is completely lacking at other points. This irregular distribution naturally results in irregular hardness and porosity of the finished sintered body.

As a result of its uniform hardness and low 50 porosity, the hard metal alloys according to the

invention are particularly suitable for accurate finishing work and for accurate drawing dies and furthermore as the material used as the tips on measuring gauges or other parts subjected to much wear on machines and apparatus. The higher acid resistance of these alloys is also frequently advantageous.

What we claim as new and desire to secure by Letters Patent of the United States, is:

1. The method of making a sintered hard metal composition which comprises mixing metal of the iron group with a compound which consists of about 1 to 5% carbon with the remainder metal from the group tungsten and molybdenum, heating said mixture to a temperature in the neighborhood of 1300° C., crushing the resulting

5 product and thereafter employing such product as a binder material for pulverized carbide particles, pressing the resulting mixture into a desired form and sintering it to thereby form a cemented carbide.

10 2. A sintered hard metal alloy which consists of one or several carbides of metals with a high melting point and a metallic addition constituting at most 25% of the total alloy, said addition having a considerably lower melting point than said carbides and consisting of a material whose combination lies within the limits indicated by the formulas  $Co_6W_2C$  and  $Co_3W_3C$ .

WALTHER DAWIHL.  
KARL SCHRÖTER.